

## UNITED STATES PATENT OFFICE

2,470,405

## CUTTING FLUID

Hollis L. Leland, Cranford, N. J., assignor to  
Standard Oil Development Company, a cor-  
poration of Delaware

No Drawing. Application December 5, 1945,  
Serial No. 633,053

1 Claim. (Cl. 252—49.8)

1

The present invention relates to cutting fluids, and more particularly to a readily water-emulsi-  
fiable composition which, in the form of an emul-  
sion, will provide a high load-carrying film be-  
tween the cutting tool and the work being ma-  
chined.

Cutting fluids are generally poured over the tool and the work in a steady stream and function to dissipate the heat from both the tool and the work; improve the quality of the surface produced; lubricate the surfaces in contact between the tool and work; prevent "build-up" on the tool or the welding of the work to the tool; to wash away the chips and to provide lubrication between the chips and the tool. For some of the foregoing purposes, such as washing away chips, any fluid will do. For dissipating heat a fluid should be provided having a high specific heat, while for improved quality of surface and long tool life, a fluid must be provided capable of supplying a high-load-carrying film.

Machining, generally speaking, is a two-stage operation, the roughing cut being the first stage and the finishing cut being the second stage. In rough cuts the primary objects is to remove material, and the quality of the surface produced is secondary. However, since in the following finishing cut only a very small amount of material is removed, the preceding rough cut should not leave the work in such a condition that the finishing cut will fail to remove the scars left by the rough cut. The effectiveness of a cutting fluid is measured by the amount of metal which can be removed during the roughing cut and yet leave the material in a condition where only a very light finishing cut need be taken. There is normally an enormous pressure between the cutting edge of the tool and the metal being machined, and in addition, due to the inherent resilience of the metal, heavy pressures are maintained between the work and the surface of the tool just over the cutting edge and between the chips and the surface of the tool just back of the cutting edge. Therefore, it is required that a cutting fluid be provided which is capable of maintaining a lubricating film even under heavy loads.

It has heretofore been recognized that the presence of sulfur and sulfur compounds improves the load-bearing characteristics of a cutting fluid. In furtherance of this idea numerous sulfur compounds and sulfurized oils have been utilized as additives in cutting fluids. In this manner cutting fluids containing as much as 8 to 10% or more of the sulfur have been developed, although usually such products contain not more than 4 to 5 per cent of sulfur. Sulfurized cutting fluids, however, leave much to be desired in their performance. Sulfur and sulfur compounds stain and corrode many non-ferrous alloys, particularly those alloys containing copper, and even

some types of iron and steel develop stain and corrosion spots after having been in contact with sulfurized cutting fluids.

Many emulsifiable metal fabricating fluids as emulsions often possess the objectionable feature of not being permanent dispersions in that they are either subject to phase separation on standing for any appreciable time or precipitate out as a sediment a large part of the ingredient present for its load-carrying characteristics. A cutting fluid having high load-bearing characteristics in the form of a stable water-emulsion is therefore quite desirable.

It is therefore an object of the present invention to produce a stable emulsion cutting fluid of high load-carrying ability. Another object is the production of a cutting fluid which will not stain or corrode either ferrous or non-ferrous alloys. These and other objects will be apparent to those skilled in the art upon reading the following description.

It has now been found that by the selection of the proper emulsifier, organic esters of acids such as phosphoric acid, phosphorous acid, thiophosphoric acid, and thiophosphorous acid or mixtures of these esters and mineral lubricating oil can be emulsified with water giving permanently stable emulsions which are useful as cutting fluids. These organic esters of the acids of phosphorus have been recognized as having oiliness or load-bearing characteristics and solutions or suspensions of them have been employed in an attempt to utilize these properties. Esters falling within these two classifications have the most probable formulae:



40 where X is either oxygen or sulfur and R is either hydrogen, an aliphatic hydrocarbon radical such as methyl, ethyl, propyl, butyl, isobutyl, octyl, decyl, dodecyl, etc.; or an aromatic hydrocarbon radical such as phenyl, cresyl, xylensyl, etc.; at least one of the R's being a hydrocarbon radical. The emulsifiers found to be particularly adapted to the emulsification of phosphoric, phosphorous, thiophosphoric and thiophosphorous acid esters in water are esters of partially dehydrated hexahydric alcohols in which the esterifying radical contains from 8-30 carbon atoms mixed with the reaction product of the same type of ester and ethylene oxide. Oleic acid ester of partially dehydrated sorbitol is illustrative of the former type of emulsifying agent, and the reaction product of palmitic acid ester of partially dehydrated sorbitol and ethylene oxide is representative of the latter type of emulsifying agent. The reaction product of the ester with ethylene oxide results in a material falling within the general class of ether-

50

55

ester compounds. In making up the emulsifier considerable latitude can be taken with respect to the ratio of ester compound to ether-ester compound. However, according to the present invention it is preferred to use these materials in the ratios of one part by weight of ester to one to three parts or more by weight of the ether-ester compound.

The ester types of emulsifying agents employed in the present invention are carboxylic acid esters of partially dehydrated aliphatic polyhydric alcohols such as the hexitols. Partial dehydration converts the polyhydric alcohol to an epoxide or inner ether type of compound having hydroxyl substituents and either one or two mono-oxy, 4-7 membered carbon-oxygen rings in its probable chemical configuration. In the case of sorbitol, monodehydration forms a sorbitan, whereas di-dehydration yields a sorbitide. The hydroxyl groups attached to the inner ethers still retain the typical reaction of an alcohol, one of which is that of reaction with a fatty acid to produce an ester. The esterification of one or more hydroxyl groups in the partially dehydrated polyhydric alcohol yields esters found to be useful for the purposes of the present invention. The acids useful for the esterification of the cyclic ether-alcohol compounds, are those fatty acids which are present combined with glycerine in naturally occurring animal and vegetable oils and fats and which are derived therefrom upon saponification thereof and are exemplified by the fatty acids derived from stearin, whale oil, menhaden oil, neat's-foot oil, castor oil, corn oil, cottonseed oil, coconut oil, linseed oil, palm kernel oil, rapeseed oil, China-wood oil, perilla oil, soya bean oil, sunflower oil, olive oil and the like and includes fatty acids, such as caproic, caprylic, capric, lauric, myristic, palmitic, oleic, linoleic, linolenic, ricinoleic, stearic, dihydroxystearic, eleostearic, erucic, and behenic. Also fatty acids such as synthetically prepared aliphatic monocarboxylic fatty acids, as for instance margaric or fatty acids prepared by suitably oxidizing hydrocarbons or by hydrogenating naturally occurring fatty acids, may be used. The naphthenic acids recovered from certain petroleum oils are also eminently satisfactory. It is also contemplated that mixtures of the foregoing acids may be used in the esterification of the partially dehydrated polyhydric alcohols.

The esters are made by reacting 1 mol of the polyhydric alcohol or 1 mol of the partially dehydrated alcohol with one to three mols of carboxylic acid or carboxylic acid mixtures either in the presence of or absence of a catalyst. The catalyst may be acidic, for example, sulfuric or phosphoric acid, or alkaline, like sodium hydroxide. The ingredients are comingled and heated in a kettle or other container, preferably closed and equipped with suitable agitating means at a temperature of 150-300° C. until the reaction

reaches the desired stage. It is frequently desirable to maintain an atmosphere of inert gas such as nitrogen or carbon dioxide over the reacting mass as by passing an inert gas over or through the reacting mass in order to assist removal of the water of condensation and prevent discoloration of the esters formed or the reaction may be carried out in a refluxing hydrocarbon solvent, with means provided for trapping out the water formed.

The ether-ester type of emulsifier is made by reacting an ester produced as above-described with an olefin epoxide such as ethylene oxide in the following manner.

The ester and 1-5% of a catalyst such as stannic chloride, are placed in a kettle or other container equipped with an suitable agitating device and means of cooling the reaction mixture to prevent the temperature rising above the boiling point of the olefin epoxide used. The desired amount of olefin epoxide is then added slowly with stirring, about one to two mols of olefin epoxide being used for each mol of ester. After about one hour the reaction is substantially complete. The catalyst may then be conveniently removed by water washing or by the use of an absorbent medium such as fuller's earth.

In making up cutting fluid emulsions, from 0.1-15% or more, being weight per cent based upon the total composition, of the phosphorus compound, will be used, and from 2-10 weight per cent of the emulsifier, the remainder of the cutting fluid being water. The emulsion is made by first thoroughly mixing the phosphorus compound with the emulsifier, heating if necessary to get an intimate mixture and then incorporating this mixture in water by means of stirring or other mechanical agitation. An emulsion stable over long periods of time is thus obtained.

In cases where the ester portion of the emulsifier is a material with a melting point above room temperature, such as occurs in the case of the ester of stearic acid, it may be necessary to form the cutting fluid by incorporating the homogeneous concentrate at 140° F.-150° F. in a small amount of water heated to a temperature above the melting point of the ester to form a concentrated emulsion. This concentrated emulsion can then be diluted with either hot or cold water to attain the desired concentration of active ingredients in the final emulsion, which will be permanently stable. Experience has shown that emulsions which do not separate within 24 hours will be permanently stable.

In the event that foaming troubles are experienced with any of the emulsions, small amounts of foam inhibitors may be added, for example, about 0.05% to 0.1% of montan or candelilla wax or 0.005% to 0.01% of a polymerized silicone.

The data included in the following table demonstrate the stability and load-carrying capacity of emulsions of this type:

| Emulsion                                                                                       | Length of Storage Without Emulsion Separation | Almen Test      |                 |
|------------------------------------------------------------------------------------------------|-----------------------------------------------|-----------------|-----------------|
|                                                                                                |                                               | Gradual Loading | Shock Loading   |
| 2% Tricresyl phosphate, 2% Emulsifier, <sup>1</sup> 2% Emulsifier, <sup>2</sup> 94% Water      | Hours                                         | 24              | Carries 15 wts. |
| 10% Tricresyl phosphate, 2.5% Emulsifier, <sup>1</sup> 2.5% Emulsifier, <sup>2</sup> 85% Water |                                               | 24              | do              |
| 2% Tricresyl phosphate, 2% Emulsifier, <sup>1</sup> 2% Emulsifier, <sup>2</sup> 94% Water      |                                               | 24              | do              |
| 10% Mineral Oil Concentrate, <sup>3</sup> 90% Water                                            |                                               | 24              | 15 weights.     |
|                                                                                                |                                               |                 | Carries 3 wts.  |

<sup>1</sup> Oleic acid ester of partially dehydrated sorbitol.

<sup>2</sup> Reaction product of palmitic acid ester of partially dehydrated sorbitol and ethylene oxide.

<sup>3</sup> Lauric acid ester of partially dehydrated sorbitol.

<sup>4</sup> Reaction product of oleic acid ester of partially dehydrated sorbitol and ethylene oxide.

<sup>5</sup> Mineral oil (40 seconds Vis. at 210° F.), 9.5% sodium sulfonate and 2.8% sodium naphthenate.

In the present invention mineral oils can also be used in conjunction with the phosphorus compounds to give a highly effective cutting fluid of the soluble oil type. A wide range of lubricating oils may be employed as the base for the cutting fluid or soluble oil, and, in general, the base oil will comprise an oil having a viscosity at 100° F. in the range of from about 90-500 seconds, an A. P. I. gravity of 23°-33° and a flash point above 300° F. However, in preparing the compositions of the present invention it is preferred to use a light coastal oil as a base, that is one having an A. P. I. gravity in the range of 25°-31° and a viscosity at 100° F. of from 100-300 seconds.

As will be explained subsequently, the mineral oil, phosphorus compound and emulsifier are first blended into a concentrate which will easily emulsify in water to give a permanent emulsion. The mineral lubricating oil will compose from 60-80 weight per cent of the concentrate, which, since it is contemplated using approximately 10 parts of concentrate in 90 parts of water, will result in a water emulsion containing from 6-8 per cent of mineral oil. In the event that mineral lubricating oil is included in the cutting fluid, it has been found necessary to use as the emulsifier those ester and ester-ether blends in which the ratio of ether-ester to ester is in the upper portion of the range previously indicated, that is to say the ratio of ether-ester to ester will be in the neighborhood of 3 parts or more of ether-ester to 1 part of ester. Also when including oil in the composition particular care must be taken in compounding the ingredients in order that a permanent emulsion will result.

A permanent emulsion can be secured by first placing the phosphorus compound, emulsifier, and oil in a kettle equipped with a stirrer and heating while stirring to 120° F. The stirring and heating are continued until a homogeneous solution is obtained. If in following this procedure difficulty is encountered in attaining homogeneity, a trace of water may be added as a solubilizer and a homogeneous solution will result. The solution thus formed can be, with or without cooling, stirred into water to yield a permanent emulsion. Ordinarily 10 parts by weight of the solution is incorporated in 90 parts by weight of water to give a cutting fluid although more or less of the solution can be employed in accordance with the needs of the particular cutting operation.

The following data illustrate the load-carrying capacity of emulsions which contain mineral lubricating oil.

| Emulsion                                   | Almen Test      |               |
|--------------------------------------------|-----------------|---------------|
|                                            | Gradual Loading | Shock Loading |
|                                            | Wt.             | Wt.           |
| Control <sup>1</sup>                       | 3               | 15            |
| 10% Concentrate A <sup>2</sup> , 90% Water | 15              | 15            |
| 10% Concentrate B <sup>3</sup> , 90% Water | 15              | 15            |

<sup>1</sup> 10% Mineral Oil concentrate (Mineral oil plus 9.5% sodium sulfonate and 2.9% sodium naphthenate), 90% Water.

<sup>2</sup> 10% Tricresyl phosphate, 8% Oleic acid ester of partially dehydrated sorbitol, 15% Reaction product of palmitic acid ester of partially dehydrated sorbitol and ethylene oxide, 70% Mineral oil (40 Seconds Vis. at 210° F.).

<sup>3</sup> 9.6% Tricresyl phosphate, 4.8% Lauric acid ester of partially dehydrated sorbitol, 18.1% Reaction product of oleic acid ester of partially dehydrated sorbitol and ethylene oxide, 67.5% Mineral oil (40 Seconds Vis. at 210° F.).

NOTE.—The Almen test was conducted as described in U. S. Patent 2,001,861, issued to J. O. Almen.

The soluble oil cutting fluids of the present invention were compared with a conventional soluble oil cutting fluid to determine corrosiveness by means of the Gooch crucible test. The Gooch crucible corrosion test consists of placing metal turnings in a Gooch crucible and pouring warm emulsion over the turnings, and after the emulsion has drained off, allowing the turnings to stand for 24 hours and noting the extent of corrosion at the end of that period. The emulsion is heated to 140°-150° F. before being poured into the crucible. In the present series of tests extremely dilute emulsions were used for the purpose of accentuating any tendency on the part of the emulsions to corrode iron or steel. The results obtained were as follows:

#### Gooch crucible corrosion test

| Emulsion Base                                                                                                                                                      | Water/Cutting Oil Ratio |                   |          |       |      |       |
|--------------------------------------------------------------------------------------------------------------------------------------------------------------------|-------------------------|-------------------|----------|-------|------|-------|
|                                                                                                                                                                    | 50/1                    | 100/1             | 50/1     | 100/1 | 50/1 | 100/1 |
|                                                                                                                                                                    | On Cast Iron            | On Malleable Iron | On Steel |       |      |       |
| Mineral Oil Concentrate <sup>1</sup> , 10% Tricresyl phosphate, 8% Emulsifier, <sup>2</sup> 15% Emulsifier, <sup>3</sup> 70% Mineral Oil (40 Sec. Vis. at 210° F.) | 3                       | 3                 | 3        | 4     | 0    | 0     |
|                                                                                                                                                                    | 3                       | 3                 | 3        | 4     | 1    | 1     |

<sup>1</sup> Mineral oil (40 seconds Vis. at 210° F.) plus 9.5% sodium sulfonate and 2.9% sodium naphthenate.

<sup>2</sup> Oleic acid ester of partially dehydrated sorbitol.

<sup>3</sup> Reaction product of palmitic acid ester of partially dehydrated sorbitol and ethylene oxide.

NOTE.—0=No rust, 1=Trace of rust, 2, 3 and 4=increasing extent of rust.

40 What is claimed is:

A water emulsifiable cutting oil consisting of approximately 70 parts by weight of mineral base oil, 5 parts by weight of oleic acid ester of partially dehydrated sorbitol, 15 parts by weight of the reaction product of palmitic acid ester of partially dehydrated sorbitol with ethylene oxide and 10 parts by weight of tricresyl phosphate.

HOLLIS L. LELAND.

#### REFERENCES CITED

The following references are of record in the file of this patent:

55

#### UNITED STATES PATENTS

| Number       | Name     | Date          |
|--------------|----------|---------------|
| 2,245,649    | Caprio   | June 17, 1941 |
| 2,328,540    | Hochwalt | Sept. 7, 1943 |
| 60 2,402,373 | Cordero  | June 18, 1946 |

#### OTHER REFERENCES

"Spans and Tweens," publication of Atlas Powder Co., 1942, pages 1-16.

65

70